

# United States Patent Office

3,220,866

Patented Nov. 30, 1965

1

3.220.866

## **CORROSION INHIBITION**

Arnold Joseph Rosenthal, Whippany, N.J., assignor to  
Celanese Corporation of America, New York, N.Y., a  
corporation of Delaware

No Drawing. Filed May 25, 1962, Ser. No. 197,595  
21 Claims. (Cl. 106—181)

The present invention relates to the prevention of corrosion of metals by solutions of organic acid esters of cellulose in halogen-containing organic solvents. More particularly, it relates to novel processes for preventing such corrosion by incorporation in the solution of special stabilizing agents.

In the course of converting organic acid esters of cellulose to filamentary material and the like, these esters may be dissolved in halogen-containing organic solvents. By way of illustration, cellulose triacetate is dissolved in methylene chloride which may also contain minor amounts of co-solvents for the ester such as methanol, ethanol, isopropanol or the like, as well as small amounts of water. This solution or dope is then dry spun into filamentary cellulose triacetate, the solvent being evaporated by a current of warm air followed by recovery and purification prior to re-use. The spinning is effected by passage of the solution through one or more orifices in a metallic member generally referred to as a jet. It has been found that these jets, as well as other metal equipment contacted by the solvent during use and recovery, corrode rapidly and require frequent replacement.

It is accordingly an object of the present invention to minimize or prevent this corrosion of metallic members contacted by halogen-containing organic solvents for organic acid esters of cellulose.

Another object is to provide a solution of cellulose triacetate in methylene chloride, which solution can be dry spun without rapid corrosion of the spinning jet.

A further object of the invention is to provide a cellulose triacetate solution which is sufficiently non-corrosive on metals to permit spinning through stainless steel jets. Other objects of this invention will be apparent from the following detailed description and claims.

In accordance with one aspect of the present invention, to a halogen-containing organic solvent solution of the organic acid ester of cellulose there is added a stabilizer or mixture of stabilizers which inhibits corrosion of metallic members. The stabilizers must satisfy certain requirements in order to be suitable for use, viz., they must themselves be non-corrosive, they should not have any particular affinity for the cellulose ester lest they contaminate articles produced therefrom, they should not deleteriously affect the physical properties of the cellulose esters, under conditions of use they should not endanger the operators, they should not irritate or sensitize the skin when worn and preferably they should be sufficiently inexpensive so that their cost will be compensated for by savings in the replacement cost of metal equipment or by improvements in the properties of the esters as a result of elimination of metallic contaminants.

The quest for suitable stabilizers is complicated by the fact that the exact mechanism of the corrosion is not fully understood. While it might be expected that the corrosion is the result of the presence of hydrohalic acids, stabilizers heretofore used to prevent corrosion in other systems or to bind any decomposition products of halogen-containing systems, e.g., organometal salts or acid binding agents such as triethylamine and triethanolamine, are ineffective in the instant situation. Moreover, the corrosion of the spinning jets is apparently independent of temperature, whereas if the corrosion were the result of decomposition with evolution of hydrogen halide it would be expected to be temperature-dependent.

2

It might also be theorized that the corrosion is due to oxidation but faces of jets exposed to air are even less corroded than those shielded from air. In addition, anti-oxidants such as hydroquinone ethers do not exert any appreciable inhibitory effect on solutions of the character herein set forth.

It has now been found that if an organotin derivative of a carboxylic acid is incorporated into a solution of an organic acid ester of cellulose in a halogen-containing organic solvent, the corrosion of metal jets from such solution is markedly reduced or, indeed, virtually eliminated. The carboxylic acid from which the organotin derivative is formed may be either a mono carboxylic acid, e.g., acetic acid, butyric acid, caproic acid, lauric acid, palmitic acid, oleic acid, behenic acid, etc., or a dicarboxylic acid, e.g., maleic acid, fumaric acid, etc.

An example of a suitable organotin derivative of a mono carboxylic acid is a dibutyltin dilaurate. Suitable derivatives of dicarboxylic acids include alkyltin maleates wherein the alkyl group contains from about 2 to 10 carbon atoms. We have found that dibutyltin maleate is particularly suitable.

In addition, organotin derivatives of mixed maleic acid and a mono carboxylic acid are also suitable. Such mixed organotin derivatives are described in U.S. Patent 2,826,597, and may be illustrated by the following structural formula:



wherein R is an alkyl, aryl or aralkyl group, and R' is an alkyl radical. Thus R may be any organic radical such as methyl, ethyl, propyl, butyl, lauryl, phenyl, benzyl, etc. Similarly, R' may be derived from any monobasic aliphatic acid such as acetic, butyric, caproic, lauric, palmitic, oleic, behenic, etc.

40 We have found that the use of one of the foregoing organotin derivatives of a carboxylic acid is extremely effective in preventing corrosion of metal jets in a dynamic situation, i.e., under actual spinning conditions. This result is quite unexpected because when such an organotin derivative of a carboxylic acid is incorporated into a spinning solution and such solution is caused to contact a metal specimen under static conditions, i.e., where-in the metal specimen is simply placed into the spinning solution, no particular inhibition to corrosion is apparent. Thus, although the explanation of the unexpected efficacy of the organotin derivatives of a carboxylic acid 45 in preventing corrosion under dynamic situations and not under static situations is not presently understood, the fact remains that in actual spinning conditions the incorporation of such derivative markedly reduces corrosion. 50

55 The organotin derivative of a carboxylic acid will exert some beneficial action when present even in the most minute quantities. However, to obtain appreciable inhibition against corrosion, such stabilizer, when used alone, should be present in an amount at least 0.005 percent by weight of the solution. Generally, the range will be from about 0.005 to 0.5% of the solution, with a more preferred range being from about 0.01 to 0.1%. Even more than about 0.5% of stabilizer can be used, but since 60 corrosion is substantially completely eliminated with 65 lesser amounts, there is no need.

In accordance with another aspect of the invention, it has been found that if, along with such organotin stabilizer, a lower alkyl amine nitrite stabilizer and particularly a hydroxysubstituted lower alkyl amine nitrite such as 2-hydroxypropylamine nitrite is incorporated into the solution of organic acid ester of cellulose in halogen-contain-

ing solvent, a synergistic effect takes place. That is, the amount of each stabilizer required to inhibit jet corrosion from such solution is markedly reduced to about 20 percent of the amount that would be required to obtain equivalent corrosion inhibition when using either the organotin stabilizer or the lower alkyl amine nitrite alone. U.S. Patent 2,927,031 teaches the incorporation of a lower alkyl amine nitrite into a halogen-containing organic solvent solution of an organic acid ester of cellulose and further teaches that the amount of amine nitrite so incorporated may be from about 0.005 to 0.5% by weight of the solution. However, as heretofore pointed out, if an organotin stabilizer, e.g., dibutyl tin maleate, and a lower alkyl amine nitrite stabilizer, e.g., 2-hydroxypropylamine nitrite are both incorporated into such solution, the amounts of each such stabilizer may be reduced to about 20% of that required when either is used alone, i.e., from about 0.001 to 0.1% by weight of the solution. Thus, the use of the organotin stabilizer and lower alkyl amine nitrite together offers obvious economic advantages.

As has been previously pointed out, the present invention finds particular application in dynamic situations, e.g., under actual spinning conditions. Thus, without the presence of either the organotin stabilizer or a stabilizing mixture of the organotin stabilizer and lower alkyl amine nitrite stabilizer, the solution of organic acid ester of cellulose in halogen-containing solvent will induce considerable corrosion of the metal jet as such solution is spun therethrough.

The solvent of the cellulose ester solution can be any halogenated organic solvent but the preferred solvents are chlorine - substituted lower alkanes such as methylene chloride, ethylene dichloride, and the like. These may contain minor amounts of co-solvents or non-solvents for the esters, depending upon the properties desired for the composition and the subsequent treatments to which it will be subjected. When a methylene chloride solution is to be used for dry spinning, for example, the methylene chloride solvent may contain as much as 20% by weight of volatile alcohols such as methanol, ethanol, propanol, isopropanol, and the like, the percentage being based on the combined weights of methylene chloride and alcohol. Although water will decrease the solubility of the ester in the solvent, small amounts can be tolerated. The stabilizing action will be realized even in the presence of water.

Organic acid esters of cellulose which can be used are preferably the lower alkanoic acid esters such as the acetate, propionate, butyrate, acetate-propionate, acetate-butyrate, and the like. While the invention is applicable to any esters which will dissolve in the indicated solvents, excellent results are achieved when using cellulose acetate having an acetyl content in excess of about 59.5% and preferably 61.5% by weight calculated as acetic acid. Such esters are substantially fully acetylated, i.e., free of unreacted hydroxyl groups, and are hereinafter referred to as cellulose triacetate although a small residue of unreacted hydroxy groups may be present.

The present invention is particularly useful in the dry spinning of solutions of cellulose triacetate in methylene

chloride-methanol, such as are disclosed in abandoned U.S. application Serial No. 566,088, filed February 17, 1956, by Robert K. Davies and Arnold J. Rosenthal. The solutions there described comprise cellulose acetates having an acetyl value in excess of 59.5% by weight expressed as acetic acid (herein referred to as cellulose triacetate) dissolved in methylene chloride-methanol to a concentration of above 15% and preferably from 17 to 27%. The methylene chloride can range upwards from 80% of the combined weights of methylene chloride and methanol with about 90% or more preferred. These solutions generally contain small amounts of water, from about 0.3% of the weight of the solution up to the amount which will create turbidity, although preferably water is present in no more than 60% by weight of the amount which will create turbidity. The amount of water which will create turbidity will vary with the composition of the solution. With the minimum concentration of 15% by weight of cellulose triacetate in the solution and about 10% of methanol in the solvent the turbidity point will correspond to about 1.7% of water.

Following spinning, the amount of stabilizer adhered to the cellulose triacetate is extremely small and any small residual amounts will be removed during the wet treatments to which fabrics made from said filamentary materials are normally subjected.

The following examples will further illustrate my invention. Each jet was made of stainless steel, was 1 inch in diameter, and contained five holes, each 0.032 mm. in diameter. In judging the jets for damage from extrusion, a numerical rating system was used to summarize the damage as revealed by microscopic examination. The following system was employed:

|    | Nature of damage:                                     | Demerits |
|----|-------------------------------------------------------|----------|
| 35 | Pits in capillary wall                                | 1        |
|    | Nicks in hole contour at jet face                     | 1        |
|    | Rejected hole (radius enlarged 0.004 mm. at any point | 3        |
| 40 | Maximum demerits permitted per hole, not rejected     | 2        |
|    | Maximum demerits assigned per rejected hole           | 3        |

$$45 \text{ Damage score per trial, percent} = \frac{\text{total demerits} \times 100}{3 \times \text{total holes in trial}}$$

### Examples 1-3

50 Cellulose acetate having an acetyl value of 61.5% is dissolved in a mixture of 91 parts by weight of methylene chloride and 9 parts by weight of methanol to form a solution having a concentration of cellulose acetate of 22% by weight based on the weight of solvent. Varying amounts of dibutyl tin maleate or of 2-hydroxypropyl amine nitrite are incorporated into the solution, as shown in Table I. The solution is spun at a temperature of 72° C. at a rate of 1200 meters per minute linear velocity of solution through the 0.032 mm. diameter hole type 316 stainless steel jets. The results are given in Table I.

TABLE I

| Example          | Stabilizer               | Stabilizer Concentration, Percent | Hours of Extrusion | Damage Score, Percent |
|------------------|--------------------------|-----------------------------------|--------------------|-----------------------|
| A (control)----- |                          | 0.00                              | 72                 | 100                   |
| 1-----           | Dibutyl tin maleate----- | 0.01                              | 30                 | 0                     |
|                  |                          | 0.01                              | 76                 | 0                     |
|                  |                          | 0.01                              | 260                | 47                    |
|                  |                          | 0.01                              | 500                | 67                    |
| 2-----           | do-----                  | 0.03                              | 54                 | 0                     |
|                  |                          | 0.03                              | 124                | 16                    |
|                  |                          | 0.03                              | 309                | 27                    |
| 3-----           | do-----                  | 0.05                              | 500                | 40                    |
|                  |                          | 0.05                              | 72                 | 0                     |
|                  |                          | 0.05                              | 500                | 0                     |

The efficacy of the dibutyl tin maleate stabilizer in preventing jet corrosion is obvious.

TABLE II

| Example          | Stabilizer                              | Stabilizer Concentration, Percent | Hours of Extrusion | Damage Score, Percent |
|------------------|-----------------------------------------|-----------------------------------|--------------------|-----------------------|
| A (control)----- | Dibutyl tin maleate-----                | 0.00                              | 72                 | 100                   |
| 4-----           | +<br>2-hydroxypropyl amine nitrite----- | 0.01                              | 48                 | 0                     |
| B-----           | 2-hydroxypropyl amine nitrite-----      | 0.01                              | {<br>169<br>500    | 0<br>7                |
| C-----           | do-----                                 | 0.005                             | 42                 | 67                    |
| D-----           | do-----                                 | 0.015                             | 500                | 87                    |
|                  |                                         | 0.025                             | 406                | 7                     |
|                  |                                         | 0.025                             | 426                | 7                     |
|                  |                                         | 0.025                             | 500                | 33                    |

*Example 4*

The procedure described in Examples 1-3 was utilized, however, both dibutyl tin maleate and 2-hydroxypropyl amine nitrite were used as stabilizers. The results are given in Table II, and are compared with the use of either dibutyl tin maleate alone (Examples 1-3), or the use of 2-hydroxypropylamine nitrite (Examples B, C and D) alone.

From the foregoing it will be seen that when 0.01 percent dibutyl tin maleate is used along with 0.01 percent 2-hydroxypropylamine nitrite, the corrosion inhibition is superior to that obtained using dibutyl tin maleate alone (e.g., Example 3, wherein 0.03% dibutyl tin maleate showed a damage score of 40 after 500 hours), and is also superior to the corrosion inhibition obtained using 2-hydroxypropylamine nitrite alone (e.g., Example D, wherein 0.025% 2-hydroxypropylamine nitrite showed a damage score of 33 after 500 hours).

The foregoing spinning solutions of my invention may be spun and the solvent recovered therefrom with little or no corrosion of metal equipment contacted therewith.

It is to be understood that the foregoing detailed description is given merely by way of illustration and that many variations may be made therein without departing from the spirit of my invention.

Having described my invention what I desire to secure by Letters Patent is:

1. A stable composition of matter, non-corrosive on metals contacted therewith, comprising a solution in a halogen-containing organic solvent of a lower alkanic acid ester of cellulose and a small amount sufficient to substantially inhibit the corrosion of metals of an organotin carboxylate, said carboxylate also being itself non-corrosive to metals, not having any particular affinity for said cellulose ester, and not deleteriously affecting the physical properties of said cellulose ester.

2. The composition of claim 1 wherein said organotin carboxylate is an alkyl tin maleate, wherein the alkyl group contains from about 2 to 10 carbon atoms, and wherein said alkyl tin maleate is present in an amount equal to at least 0.005% by weight of said solution.

3. A stable composition of matter, non-corrosive to spinnerets contacted therewith in a spinning process, comprising a solution of cellulose triacetate in a concentration of at least 15% by weight in a solvent comprising methylene chloride and a lower alkanol, the methylene chloride constituting at least about 80% by weight of the solvent, said solution containing about 0.005 to 0.5% by weight and sufficient to substantially inhibit the corrosion of metals of an alkyl tin maleate wherein the alkyl groups contain 2 to 10 carbon atoms as stabilizer, said maleate also being itself non-corrosive to metals, not having any particular affinity for said cellulose ester, and not deleteriously affecting the physical properties of said cellulose triacetate.

4. A stable composition of matter, non-corrosive to spinnerets contacted therewith in a spinning process, comprising a solution of cellulose triacetate in a concentration ranging from about 17 to 27% by weight in a solvent comprising about 90% by weight of methylene chloride

and about 10% by weight of methanol, said solution containing water in an amount between a minimum of about

0.3% by weight and a maximum of the amount which will bring the solution to the turbidity point, said solution further containing about 0.005 to 0.5% by weight and sufficient to substantially inhibit the corrosion of metals of an alkyl tin maleate wherein the alkyl groups contain 2 to 10 carbon atoms as stabilizer, said maleate also being itself non-corrosive to metals, not having any particular affinity for said cellulose ester, and not deleteriously affecting the physical properties of said cellulose triacetate.

5. A stable composition of matter, non-corrosive to metallic spinnerets contacted therewith in a spinning process, comprising a solution in a halogen-containing organic solvent of a lower alkanic acid ester of cellulose and a small amount sufficient to substantially inhibit the corrosion of metals of an alkyl tin maleate wherein the alkyl groups contain 2 to 10 carbon atoms and of a hydroxy lower alkyl amine nitrite, said maleate and nitrite also being themselves non-corrosive to metals, not having any particular affinity for said cellulose ester, and not deleteriously affecting the physical properties of said cellulose ester.

6. The composition of claim 5 wherein said alkyl tin maleate and said hydroxy lower alkyl amine nitrite are each present in an amount equal to from about 0.001 to 0.1% by weight of said solution.

7. A stable composition of matter, non-corrosive to metallic spinnerets contacted therewith in a spinning process, comprising a solution of cellulose triacetate in a concentration of at least 15% by weight in a solvent comprising methylene chloride and a lower alkanol, the methylene chloride constituting at least about 80% by weight of the solvent, said solution containing about 0.001 to 0.1% by weight and sufficient to substantially inhibit the corrosion of metals of each of an alkyl tin maleate wherein the alkyl groups contain 2 to 10 carbon atoms and a hydroxy lower alkylamine nitrite, said maleate and nitrite being themselves non-corrosive to metals, not having any particular affinity for said cellulose triacetate, and not deleteriously affecting the physical properties of said cellulose triacetate.

8. A stable composition of matter, non-corrosive to metallic spinnerets contacted therewith in a spinning process, comprising a solution of cellulose triacetate in methylene chloride, said solution containing a small amount sufficient to substantially inhibit the corrosion of metals of 2-hydroxypropylamine nitrite and of dibutyl tin maleate, said maleate and nitrite being themselves non-corrosive to metals, not having any particular affinity for said cellulose triacetate, and not deleteriously affecting the physical properties of said cellulose triacetate.

9. A process for stabilizing a solution against corrosion of metal contacted therewith, said solution comprising a lower alkanic acid ester of cellulose dissolved in a halogen-containing organic solvent, which process comprises incorporating a small amount sufficient to substantially inhibit the corrosion of metals of an organotin carboxylate in said solution, said carboxylate also being itself non-corrosive to metals, not having any particular

affinity for said cellulose ester, and not deleteriously affecting the physical properties of said cellulose ester.

10. A process for stabilizing a solution against corrosion of metal contacted therewith, said solution comprising cellulose triacetate dissolved in methylene chloride, which process comprises incorporating a small amount sufficient to substantially inhibit the corrosion of metals of dibutyl tin maleate in said solution, said maleate also being itself non-corrosive to metals, not having any particular affinity for said cellulose ester, and not deleteriously affecting the physical properties of said cellulose triacetate.

11. The process of claim 9 wherein said stabilizing proportion is from about 0.005 to 0.5% by weight of said solution.

12. In the production of filamentary material wherein a solution of a lower alkanoic acid ester of cellulose in a halogen-containing organic solvent is extruded through an orifice in a metallic member under conditions such that said cellulose ester is converted to filamentary material, the improvement which comprises incorporating in said solution a small amount of an organotin carboxylate, whereby corrosion of said metallic member and transfer of metal to said solution and said filamentary material are inhibited, said carboxylate also being itself non-corrosive to metals, not having any particular affinity for said cellulose ester, and not deleteriously affecting the physical properties of said cellulose ester.

13. The process of claim 12 wherein said stabilizing proportion is from about 0.005 to 0.5% by weight of said solution.

14. The process for stabilizing a solution against corrosion of metal contacted therewith, said solution comprising a lower alkanoic acid ester of cellulose dissolved in a halogen-containing organic solvent, which process comprises incorporating a small amount sufficient to substantially inhibit the corrosion of metals of a hydroxy lower alkyl amine nitrite and of an alkyl tin maleate wherein the alkyl groups contain 2 to 10 carbon atoms, said maleate and nitrite also being themselves non-corrosive to metals, not having any particular affinity for said cellulose ester, and not deleteriously affecting the physical properties of said cellulose ester.

15. The process of claim 14 wherein the hydroxy lower alkyl amine nitrite is 2-hydroxypropylamine nitrite and wherein said alkyl tin maleate is dibutyl tin maleate.

16. In the production of filamentary material wherein a solution of a lower alkanoic acid ester of cellulose in a

halogen-containing organic solvent is extruded through an orifice in a metallic member under conditions such that said cellulose ester is converted to filamentary material, the improvement which comprises incorporating in said solution a small amount of a hydroxy lower alkyl amine nitrite and of an alkyl tin maleate wherein the alkyl groups contain 2 to 10 carbon atoms, whereby corrosion of said metallic member and transfer of metal to said solution and said filamentary material are inhibited, said maleate and nitrite also being themselves non-corrosive to metals, not having any particular affinity for said cellulose ester, and not deleteriously affecting the physical properties of said cellulose ester.

17. The process of claim 16 wherein the hydroxy lower alkyl amine nitrite is 2-hydroxypropylamine nitrite and wherein said alkyl tin maleate is dibutyl tin maleate.

18. The process of claim 16 wherein said stabilizing proportion for said hydroxy lower alkyl nitrite is from about 0.001 to 0.1% and wherein said stabilizing proportion for said alkyl tin maleate is from 0.01 to 0.1% by weight of said solution.

19. The composition of claim 1 wherein said organotin carboxylate is dibutyltin dilaurate.

20. The composition of claim 1 wherein said organotin carboxylate is a compound of the formula:



wherein R is selected from the group consisting of alkyl, aryl and aralkyl, and wherein R' is alkyl.

21. The process of claim 12 wherein said ester of cellulose is cellulose triacetate and said halogen-containing organic solvent comprises methylene chloride.

#### References Cited by the Examiner

##### UNITED STATES PATENTS

|           |         |           |       |         |
|-----------|---------|-----------|-------|---------|
| 2,826,597 | 3/1958  | Gloskey   | ----- | 260—429 |
| 2,857,413 | 10/1958 | Weinberg  | ----- | 260—429 |
| 2,927,031 | 3/1960  | Rosenthal | ----- | 106—186 |

45 ALEXANDER H. BRODMERKEL, *Primary Examiner.*  
MORRIS LIEBMAN, *Examiner.*